

J. W. HOWELL.  
 METHOD OF FUSING LAMP FILAMENTS TO LEADING-IN WIRES.  
 APPLICATION FILED MAR. 16, 1907.  
**1,022,553.** Patented Apr. 9, 1912.



Witnesses:

Peter H. Fulmer.  
 J. Ellis Van.

Inventor,  
 John W. Howell,  
 By *Albert H. Davis*  
 Atty.

# UNITED STATES PATENT OFFICE.

JOHN W. HOWELL, OF NEWARK, NEW JERSEY, ASSIGNOR TO GENERAL ELECTRIC COMPANY, A CORPORATION OF NEW YORK.

## METHOD OF FUSING LAMP-FILAMENTS TO LEADING-IN WIRES.

1,022,553.

Specification of Letters Patent.

Patented Apr. 9, 1912.

Application filed March 16, 1907. Serial No. 362,610.

*To all whom it may concern:*

Be it known that I, JOHN W. HOWELL, a citizen of the United States, residing at Newark, county of Essex, State of New Jersey, have invented certain new and useful Improvements in Methods of Fusing Lamp-Filaments to Leading-In Wires, of which the following is a specification.

Incandescent lamp filaments consisting of 10 a refractory metal, such as tungsten, molybdenum, boron, titanium, etc., may be advantageously supplied with current through a leading-in conductor fused or welded to the filament. Such a joint affords a rigid connection of good conductivity and free from 15 any carbonaceous or other vaporizable material which might contaminate the filament. Such a welded connection can be made to a platinum leading-in wire by 20 means of an electric arc in a non-oxidizing atmosphere. The platinum leading-in wire fuses into a globule and appears to alloy or otherwise combine with the tungsten of the filament.

25 According to my present invention the filament is connected by a welding or fusing operation with a leading-in conductor or wire consisting of a metal or material which does not readily alloy or combine 30 with the material of the filament. When the two materials are of this nature, there is no danger that the fused globule will soak into the filament and possibly change its refractory qualities in immediate proximity 35 to the welded joint. According to the process hereinafter described, a large proportion of perfect joints are obtainable and the welding or fusing operation is performed in such a manner that the filaments are protected from the deteriorating action of the 40 welding arc.

According to my invention, the leading-in conductor or supporting wire to which the filament is to be connected is provided with 45 a thin tubular portion bent downward to form a socket for the reception of the end of the filament. The fusing arc is drawn from the lower end of the tubular socket and therefore at some distance from the 50 filament, or more strictly speaking, at some distance from the portion of the filament operating at incandescence when the lamp is in use.

The details of my invention will be better

understood by reference to the accompanying drawing, in which—

Figure 1 is a sectional elevation of an apparatus suitable for carrying out the welding operation; Fig. 2 is an enlarged view of the joint before the arc is formed; 60 and Fig. 3 is an enlarged view of the finished connection.

The welding operation may be carried out in a glass envelop 1 provided at the top with an inlet 2 through which hydrogen or 65 other non-oxidizing gas may be continuously supplied. The envelop may be open at the bottom for the convenient introduction of a lamp stem 3 carrying a pedestal 4 about which the several metal filaments 5 70 are grouped. These filaments may consist of pure tungsten or of other refractory metals and materials. Leading-in conductors or support wires 6 of copper or other suitable metal, may be arranged axially 75 about the pedestal 4, as shown in the drawing. Before assembling the lamp, each leading-in wire is flattened at the end and then drawn through a die to shape the flattened portion into a tube 7, as illustrated 80 in Fig. 2. This tube is bent downward at a substantially right angle to the leading-in conductor and thus serves as a convenient socket for the end of a lamp filament 5.

The order of procedure is as follows: 85 The leading-in conductor is placed in the notched end of a rod 8 which projects through an opening in the wall of the glass envelop 1, and is connected to a source of energy 9. This rod serves to conduct the 90 arc-producing current. An electrode 10 of carbon, metal, or other suitable material is connected with the other terminal of the source and is movable through an opening 11 in the wall of the envelop. To produce 95 the weld, the carbon electrode is brought in contact with the lower end of the tubular socket 7 and is then quickly withdrawn to produce a heating arc. The lower end of the tube quickly fuses up and gathers in a 100 globule about the metal filament and then solidifies. The upper end of the tube is preferably left unfused, for it then acts as an anchor for the filament during the welding operation, and so keeps the filament centrally located in the fused part. Unless the filament is thus anchored, it may move 105 entirely out of the globule. Owing to the

distance between the carbon electrode and the filament, the latter is not subjected to the deteriorating action of the arc.

It is of great importance to select for the 5 leading-in wire, a material which does not alloy or combine with the material of the filament,—as for instance, copper wire for tungsten filaments. No flux is used and the fused portion of the copper conductor re-10 mains unalloyed.

What I claim as new, and desire to secure by Letters Patent of the United States, is,—

1. The process which consists in rigidly securing a tungsten lamp filament to a copper support and then fusing a portion of 15 said support to form a connection of good conductivity, leaving unfused a portion of said support to which said filament is secured, said unfused portion of said support being adjacent the operative part of 20 said filament.

2. In an incandescent lamp, the combination of a tungsten filament, and a copper leading-in wire having a portion fused 25 about said filament and an unfused portion supporting the filament.

3. The method which consists in fusing a portion of a metallic member about a refractory filament of material which does 30 not readily combine with that of said mem-

ber, to form a conductive joint while the filament is maintained by another portion of said member in a position where it will be inclosed in the fused metal.

4. The method which consists in fusing 35 the end of a copper member about a tungsten filament to form a conductive joint while the filament is maintained in proper relation to the fused end of the member by another portion thereof.

5. The combination with a refractory filament of a current conductor of material inert with respect to that of the filament loosely embracing one portion thereof and fused about a portion of the filament farther 45 from the principal luminous portion than the portion thus embraced.

6. In an incandescent lamp the combination of a tungsten filament and a support wire therefor having a bent portion surrounding a part of the filament next to the operating portion thereof and fused about the filament at a point away from the operating portion of the filament.

In witness whereof, I have hereunto set 55 my hand this 8th day of March, 1907.

JOHN W. HOWELL.

Witnesses:

J. HARRY ELKINS,  
S. N. WHITEHEAD.